# EUROPEAN PATENT SPECIFICATION

(11) **EP 0 268 594 B1**
(45) Date of publication and mention of the grant of the patent: **23.01.1991**
(21) Application number: 87902185.5
(22) Date of filing: 01.04.1987
(51) Int. Cl.: E04B 1/86

(54) **SOUND ABSORBING MINERAL WOOL PRODUCT AND METHOD OF MANUFACTURING THE SAME**
SCHALLDAEMPFENDES MINERAL-WOLLEERZEUGNIS UND DESSEN HERSTELLUNG
PRODUIT EN COTON MINERAL INSONORISANT ET PROCEDE DE FABRICATION DUDIT PRODUIT

(30) Priority: 03.04.1986 SE 8601493
(43) Date of publication of application: 01.06.1988
(73) Proprietor: ROCKWOOL AKTIEBOLAGET, S-541 86 Skövde (SE)
(72) Inventor: LUNDQUIST, Per-Olof, S-541 36 Skövde (SE)
(74) Representative: Avellan-Hultman, Olle
(86) International application number: SE8700167
(87) International publication number: WO8705960

(56) References cited:
- SE-A- 200 496
- US-A- 1 966 069
- US-A- 2 450 911
- US-A- 3 111 188

## Description

The present invention generally relates to a mineral wool product, and more particularly the invention is directed to a mineral wool product for sound absorbing purposes and a method of manufacturing such product.

Modern buildings, especially large buildings, are often provided with an extensive and sophisticated ventilation system. In buildings having such systems it is important that people in the building do not hear sounds from fans or from the flow of air in the ventilation channels. It is also important that sounds, e.g. music or conversation are not transferred from one room to another over the common ventilation channels. In order to avoid such problems it has mostly been necessary to provide some type of sound insulation in the ventilation system, e.g. by introducing some type of sound absorbing material in the ventilation channels. Basically this can be made in two different ways:
-according to one way the ventilation channels or ventilation drums are made of, or are covered with, a sound absorbing material, e.g. felt or board of mineral wool;
- according to the second way sound traps are formed in the ventilation channels or ventilation drums, e.g. by providing elements in the channels, the main object of which is to fade out or absorb sounds distributed by the air inside the channels. The sound traps, in turn, mainly can be of two different types, namely a type which deflects the ventilation air once or twice by baffles, or sound traps of in-line type, in which the air flows substantially straight linear through a channel having a substantially constant cross section area, and in which the channel walls are made of or covered with a sound absorbing material.

Especially in the latter case there are very great demands on the efficiency of the sound absorba- tion. By means of mineral wool it is possible without difficulty to obtain an effective absorba- tion of sound of fairly high frequencies, e.g. more than 1000 Hz, but a standard type of such sound absorbing material, however, has a restricted possibility of absorbing sound of low frequencies.

It is known that the ability of the mineral wool to absorb low frequence sound can be increased by giving the mineral wool a surface layer of a suitable material, e.g. a thin layer of plastic. If the plastic is sufficiently thin and elastic the ability of the mineral wool product to absorb low frequence sound is drastically increased, and still its ability of absorbing high frequence sound is not reduced by any noticable extent.

Mineral wool materials of said type having a surface covering, however, have substantial disadvantage. Firstly the plastic foils, by means of which the mineral wool is covered are inflammable, and secondly it is technically difficult to apply the plastic film on the mineral wool, especially in narrow spaces like on the concave inner surface of a tubular insulation or similar means.

From US-A-1 966 069 is known an acoustic body formed from a slurry of water glass and mineral wool. The surface of the resulting body is then ground to expose the sound absorbing porous interior.

Now it has been surprisingly proved that it is possible to obtain the same good effect as with the plastic film covering substantially more simple, quicker and more economical by a method, namely by covering the mineral wool insulation with a diluted binder solution which is then allowed to dry. Two circumstances are of determining importance concerning the amount of binder solution and the state of the binder solution:
-on one hand the amount of binder etc must be sufficient to interlock practically all fibres on the surface of the mineral wool product,
- on the other hand the amount of binder must not be so great that an integral, unbroken film of binder is formed on the surface of the mineral wool product.

Generally it is not necessary to cover the surface of the entire mineral wool product, since those surfaces, which do not directly form a part of the ventilation channel are not subjected to sound and therefore cannot absorb or fade out the sound of the ventilation channels. Therefore it is quite sufficient to treat only the surfaces of the mineral wool body which directly define the channel. It may also be suitable that some parts of the surfaces which define the channel are left untreated so that said parts can increase the ability of the material to absorb the highest frequencies of the sound.

According to the invention the actual surfaces of the mineral wool bodies are covered with a non-inflammable alkali silicate like water glsss as indicated in claims 1 and 5. A suitable water glass substance is provided by EKA under the trade name "Bindizil FK10".

The water glass is pre-polymerized to obtain a viscosity of at least 300 IPa - s at 20°C and 50% dry matter content. For technical application reasons the dry matter content must not be too large, and preferably the dry matter content is kept less than 40%, preferably less than 38%.

The amount of binder applied to the mineral wool surface is of substantial importance. On one hand the amount should be sufficient to bind all loose surface fibres, on the other hand the amount must not be so large that the binder provides an integral covering over the mineral wool body. Practical tests have proved that the amount of binder applied to the product should be between 75 and 150 g dry matter/m2 of the mineral wool surface, or preferably between 95 and 140 g/m^{2.}

Also the temperature during the drying or the evaporation of the solvent is important so that the surface covering substance should keep its pliability. Tests have shown that the temperature should not be higher than 120°C.

There are different ways of applying the binder, e.g. rolling or spraying the binder. When rolling the binder onto the mineral wool product there is, however, a risk that loose fibres stick to the roller and in time put the result of the treatment at risk. Therefore it is recommended that the binder is sprayed on to the product.

It is important that the fibres of the mineral wool material are not of a hydrophobic surface character so that said fibres make it difficult or impossible to apply the binder or to obtain a correct spreading of the binder over the surface fibres. In order to eliminate said risk the binder therefore preferably can be given a slight amount of a wetting agent, e.g. a water soluble tenside.

## Claims

1. A mineral wool body suited as a sound insulating body capable of damping or absorbing both high frequency and low frequency sound, characterized
in that at least the largest amount of the fibres of the mineral wool body which are exposed to the high frequency and low frequency sound are covered with a binder to such an extent and in such way, that practically all fibres at the surface of the mineral wool body are bound to each other without the binder forming an integral, unbroken film of binder,
in that the binder is a non-inflammable type alkali silicate water glass,
and in that said water glass is pre-polymerized.

2. Mineral wool body according to claim 1, characterized in that the water glass is applied in an amount of 75-150 or preferably 95-140 g dry matter/m2 of the mineral wool body,

3. Mineral wool body according to claim 1 or 2, characterized in that the binder contains a slight amount of a wetting agent.

4. Mineral wool body according to claim 1, 2 or 3, characterized in that the mineral wool body is in the form of disks or semi-cylindrical tubes and is provided inside a ventilation channel system and covers the entire flow area thereof.

5. Method of manufacturing mineral wool bodies, e.g. plates or semi-cylindrical tubes, according to any of the preceding claims which are capable of damping or absorbing both high frequency and low frequency sound, characterized in that a diluted solution of prepolymerized water glass is applied to the mineral wool body, whereupon the solvent of the water glass is allowed to evaporate, and whereby the binder is applied in an amount which is sufficient to bind practically all fibres at the surface of the mineral wool body after the solvent has become evaporated, without forming an integral, unbroken film of binder.

6. Method according to claim 5, characterized in that only a part of the surface of the mineral wool body, which is subjected to sound, is surface- treated.

7. Method according to claim 5 or 6, characterized in that the water glass is applied by being sprayed or rolled onto the mineral wool body.

8. Method according to claim 7, characterized in that the binder is pre-polymerized to a viscosity of more than 300 mPa - s at 20°C and a dry matter content of 50% before the binder is applied to the mineral wool body.

9. Method according to any of claims 5-8, characterized in that the water glass, before being applied to the mineral wool body, is given a concentration of less than 40% or preferably less than 38% dry matter content, and in that the binder is applied in an amount of 75-150 or preferably 95-140 g dry matter/m2 of the mineral wool body.

10. Method according to any of claims 5-9, characterized in that the solvent of the water glass is allowed to evaporate or dry at a relatively low temperature, preferably at a temperature of less than 120°C.

## Patentansprüche

1. Als Schalldämpfer geeigneter Mineralwollkörper, der Schall sowohl hoher als auch niedriger Frequenz dämpfen oder absorbieren kann, dadurch gekennzeichnet,
daß wenigstens der größte Teil der Fasern des Mineralwollköpers, die dem hoch- und niederfrequenten Schall ausgesetzt sind, mit einem Bindemittel in solchem Ausmaß und in solcher Weise überzogen sind, daß praktisch alle Fasern an der Oberfläche des Mineralwollkörpers miteinander verbunden sind, ohne daß das Bindemittel einen durchgehenden, ununterbrochenen Film bildet,
daß das Bindemittel ein nicht entflammbares Alkalisilikat-Wasserglas ist
und daß Wasserglas vorpolymerisiert ist.

2. Mineralwollkörper nach Anspruch 1, dadurch gekennzeichnet daß das Wasserglas in einer Menge von 75 bis 150 oder vorzugsweise 95 bis 140 Gramm Trockenmasse pro Quadratmeter des Mineralwollkörpers aufgebracht wird.

3. Mineralwollkörper nach Anspruch 1 oder 2, dadurch gekennzeichnet, daß das Bindemittel einen geringen Anteil eines Benetzungsmittels enthält.

4. Mineralwollkörper nach Anspruch 1, oder 3, dadurch gekennzeichnet, daß der Mineralwollkörper in Form von Scheiben oder halbzylindrischen Rohem vorliegt, im Inneren eines Belüftungskanalsystems angeordnet ist und die gesamte Strömungsfläche desselben bedeckt.

5. Verfahren zur Herstellung von Mineralwollkörpern, beispielsweise von Platten oder halbzylindrischen Rohren, nach einem der vorstehenden Ansprüche, die sowohl hoch- als auch niederfrequenten Schall zu dämpfen oder zu absorbieren vermögen, dadurch gekennzeichnet, daß eine verdünnte Lösung aus vorpolymerisiertem Wasserglas auf den Mineralwollkörper aufgetragen wird, woraufhin das Lösungsmittel aus dem Wasserglas verdampfen gelassen wird und wobei das Bindemittel in einer Menge aufgebracht wird, ausreicht, um praktisch alle Fasern an der Oberfläche des Mineralwollkörpers zu binden, nachdem das Lösungsmittel verdampft ist, ohne einen durchgehenden, ununterbrochenen Bindemittelfilm zu bilden.

6. Verfahren nach Anspruch 5, dadurch gekennzeichnet, daß nur ein Teil der Oberfläche des Mineralwollkörpers, der Schall ausgesetzt ist, oberflächenbehandelt wird.

7. Verfahren nach Anspruch 5 oder 6, dadurch gekennzeichnet, daß das Wasserglas durch Sprühen oder Rollen auf den Mineralwollkörper aufgebracht wird.

8. Verfahren nach Anspruch 7, dadurch gekennzeichnet, daß das Bindemittel auf eine Viskosität von mehr als 300 mPa - s bei 20°C und einen Trockenmassegehalt von 50% vorpolymerisiert wird, bevor das Bindemittel auf den Mineralwollkörper aufgebracht wird.

9. Verfahren nach einem der Ansprüche 5 bis 8, dadurch gekennzeichnet, daß das Wasserglas vor dem Aufbringen auf die Mineralwolloberfläche auf eine Konzentration von weniger als 40% oder vorzugsweise weniger als 38% Trockenmassegehalt gebracht wird und daß das Bindemittel in einer Menge von 75 bis 150 oder vorzugsweise 95 bis 140 Gramm Trockenmasse pro Quadratmeter Mineralwollkörper aufgebracht wird.

10. Verfahren nach einem der Ansprüche 5 bis 9, dadurch gekennzeichent, daß das Lösungsmittel aus dem Wasserglas bei relativ niedriger Temperatur, vorzugsweise bei einer Temperatur kleiner 120°C, verdampfen gelassen oder getrocknet wird.

## Revendications

1. Corps de laine minérale convenant comme corps insonorisant, pouvant atténuer ou absorber le son, tant à hautes fréquences qu'à basses fréquences, caractérisé par le fait qu'au moins la plus grande partie des fibres du corps de laine minérale qui sont exposées aux sons à haute et à basse fréquence sont recouvertes de liant dans une mesure et d'une façon telles que pratiquement toutes les fibres de la surface du corps de laine minérale soient liées les unes aux autres sans que le liant ne forme une pellicule intégrale et ininterrompue, que le liant est un verre soluble silicate d'alcali type non inflammable et que ce verre soluble est pré-polymérisé.

2. Corps de laine minérale selon la revendication 1, caractérisé par le fait que le verre soluble est appliqué à raison de 75-150, ou de préférence 95-140 grammes de matière sèche par mètre carré de corps de laine minérale.

3. Corps de laine minérale selon la revendication 1 ou la revendication 2, caractérisé par le fait que le liant contient une petite quantité d'agent mouillant.

4. Corps de laine minérale selon les revendications 1, 2, ou 3, caractérisé par le fait que le corps de laine minérale est en forme de disques ou de tubes semi-cylindriques et est installé à l'intérieur d'un système de conduits de ventilation et en recouvre toute la surface de passage.

5. Procédé de fabrication de corps de laine minérale, par exemple, plaques ou tubes semi-cylindriques, selon l'une quelconque des revendications précédentes pouvant atténuer ou absorber les sons, tant de basses fréquences que de hautes fréquences, caractérisé par le fait qu'une solution diluée de verre soluble pré-polymérisé est appliquée au corps de laine minérale, après quoi on laisse évaporer le solvant du verre soluble, le liant étant appliqué en une quantité suffisante pour lier pratitiquement toutes les fibres de la surface du. corps de laine minérale après évaporation du solvant, sans former une pellicule de liant intégrale et ininterrompue.

6. Procédé selon la revendication 5, caractérisé par le fait que seul une partie de la surface du corps de laine minérale, exposée aux bruits, reçoit ce traitement de surface.

7. Procédé selon la revendication 5 ou la revendication 6, caractérisé par le fait que le verre soluble est appliqué sur le corps de laine minérale par pulvérisation ou au moyen d'un rouleau.

8. Procédé selon la revendication 7, caractérisé par le fait que le liant est pré-polymérisé pour avoir une viscosité supérieure à 300 mPa à 20°C et une teneur en matière sèche de 50% avant d'être appliqué au corps de laine minérale.

9. Procédé selon l'une quelconque des revendications 5 à 8, caractérisé par le fait que le verre soluble, avant d'être appliqué au corps de laine minérale, est concentré à moins de 40% ou, de préférence, moins de 38% de teneur de matière sèche et que le liant est appliqué à raison de 75 à 150, de préférence, de 95 à 140 grammes de matière sèche par mètre carré du corps de laine minérale.

10. Procédé selon l'une quelconque des revendications 5 à 9, caractérisé par le fait que l'on laisse évaporer ou sécher le solvant du verre soluble à une température relativement basse, de préférence, à une température inférieure à 120°C.
